

# UNITED STATES PATENT OFFICE.

WILLIAM H. STEINBERG, OF MILWAUKEE, WISCONSIN, ASSIGNOR TO THE CUTLER-HAMMER MFG. CO., OF MILWAUKEE, WISCONSIN, A CORPORATION OF WISCONSIN.

## ELECTRICAL INSULATING COMPOSITION AND PROCESS OF MAKING THE SAME.

1,233,416.

Specification of Letters Patent. Patented July 17, 1917.

No Drawing.

Application filed August 23, 1915. Serial No. 46,976.

*To all whom it may concern:*

Be it known that I, WILLIAM H. STEINBERG, a citizen of the United States, residing at Milwaukee, in the county of Milwaukee and State of Wisconsin, have invented new and useful Improvements in Electrical Insulating Composition and Processes of Making the Same, of which the following is a full, clear, concise, and exact description.

10 This invention relates to improvements in composition of material particularly adapted for electrical insulating purposes.

In my prior application Serial No. 11,337, filed March 1, 1915, there is disclosed a composition having a base including comminuted asbestos and sulfur and a binder including coal tar pitch, stearin pitch, castor oil and benzol and also a method of combining the aforesaid ingredients.

20 This composition has proven a great success commercially and the present invention contemplates the use of the same ingredients and their equivalents but the combination thereof in a slightly different way to further 25 increase the utility of the product.

More particularly the former method provided for cold mixing of the castor oil with a preheated mixture of the two pitches and while the resultant product was readily 30 moldable in innumerable forms it exhibited a tendency to crack when molded in certain special forms and the present invention eliminates, or at least greatly minimizes, such tendency and possibly improves the 35 product in other respects not yet ascertained.

According to the present invention comminuted asbestos is employed for the base and sulfur is added thereto as in the composition mentioned, the sulfur constituting 40 what is believed to be a vulcanizing agent in the final product. The asbestos and sulfur may, of course, be used in the desired proportions but in practice it has been found advantageous to use an amount of sulfur 45 equal to two per cent. of the weight of the asbestos. The asbestos and sulfur are mixed dry prior to the addition of the binder.

Also, as in the aforesaid composition, the binder includes coal tar pitch and stearin 50 pitch, preferably in equal parts, which are mixed in the presence of heat from 400 to 500° F. until the free carbon thereof precipitates. Then while said pitches are heated, an animal or vegetable oil capable of vulcanization or polymerization, preferably 55

castor oil, is added thereto in the proportion of 10% of the combined weight of the pitches after precipitation of the carbon, although as will be understood these proportions may be varied, if desired. Then after the addition of the aforesaid oil the supernatant liquid is drawn off and cooled and a volatile solvent, preferably benzol, added thereto, which completes the binder. The percentage of benzol may, of course, be varied but an amount equal to 50% of the liquid to which it is added is usually sufficient.

Thus whereas in the formation of the binder of the former composition the benzol and castor oil were added to the supernatant liquid after cooling, the castor oil is now added before the benzol and while the pitches are still heated. Moreover, with the binder so formed, it is found that the tendency for the composition to crack when molded is materially minimized, if not entirely eliminated, while the castor oil still functions as in the former binder to stabilize the benzol, or in other words, reduce the rate of free volatilization thereof. While the theory of the improved result cannot be advanced with certainty it seems probable that the tendency of the former composition to crack resulted from the extreme greasiness of the castor oil and that by the present method the effect thereof is neutralized.

After the base and binder are completed they are mixed in a cold state as described in my prior application, preferably in the proportions of four parts of the base to one part of the binder and when mixed thoroughly they produce a granular but plastic compound. This compound may then be molded without heat and subsequently baked to produce an extremely hard and dense insulation. In molding, the material is preferably subjected to a pressure of 6,000 to 10,000 pounds per square inch and in baking the molded article is preferably subjected to a gradually increasing heat up to 450° or 500° F. and for a period of approximately twenty-four hours. As in the former composition the baking drives off by evaporation the ingredients which are volatile at the prevailing temperatures and during the baking the sulfur and the castor oil and other hemically unsatisfied constituents of the binder combine or vulcanize to yield a tough and durable insulating product which will resist heat to at least 450° to 500° F. without

softening or distorting. Also, as in the former composition, the precipitation of the free carbon of the pitches augments the effectiveness of the binder, as set forth in my prior application, aforesaid.

5. What I claim as new and desire to secure by Letters Patent is:

1. A binder for the purpose set forth, including coal tar pitch, stearin pitch and an oil capable of vulcanization or polymerization all mixed in the presence of heat.

10. 2. A binder for the purpose set forth including a preheated mixture of coal tar pitch, stearin pitch and an oil capable of vulcanization or polymerization combined with a volatile solvent.

15. 3. A composition of the character set forth including a base having mixed therewith a vulcanizing or polymerizing agent and a binder for said base including a preheated combination of coal tar pitch, stearin pitch and an oil capable of vulcanization or polymerization.

20. 4. A composition of the character set forth including comminuted asbestos and sulfur and a binder composed of a preheated combination of coal tar pitch, stearin pitch and an oil capable of vulcanization or

25. polymerization mixed with a volatile solvent.

30. 5. The herein described method consisting in combining under heat coal tar pitch, stearin pitch and an oil capable of vulcanization or polymerization.

35. 6. The herein described method consisting in combining under heat coal tar pitch, stearin pitch and an oil capable of vulcanization or polymerization and then mixing therewith when cooled a volatile solvent.

40. 7. The herein described method consisting in combining under heat coal tar pitch and stearin pitch until the free carbon thereof is precipitated and then combining therewith under heat an oil capable of vulcanization or polymerization.

45. 8. The herein described method consisting in combining under heat coal tar pitch and stearin pitch until the free carbon thereof is precipitated, then combining therewith under heat an oil capable of vulcanization or polymerization and then cooling the resultant product and adding thereto a volatile solvent.

50. In witness whereof, I have hereunto subscribed my name.

WILLIAM H. STEINBERG.